

# United States Patent Office

2,727,036

Patented Dec. 13, 1955

1

2,727,036

## HYDROCARBON OIL ADDITIVE

John P. McDermott, Springfield, N. J., assignor to Esso Research and Engineering Company, a corporation of Delaware

No Drawing. Application August 25, 1951,  
Serial No. 243,767

5 Claims. (Cl. 260—243)

The present invention relates to an improved class of 15 additives particularly suitable for use in lubricating oils and to the compounded mineral oils and other hydrocarbon products in which they are employed.

This application is a continuation-in-part of my co-pending application Ser. No. 100, 741, filed on June 22, 20 1949, now U. S. Patent No. 2,610,182.

Modern developments in the design of internal combustion engines, with increasing engine speeds and compression ratios, have imposed a severe strain on the lubricants employed. In particular, the crankcase oil is raised 25 to a high temperature and in the course of its circulation through the engine is repeatedly exposed to air under conditions highly conducive to destructive oxidation. Oxidative breakdown of the oil results in the formation of acidic products which corrode bearing surfaces and do considerable harm to the engine generally. Furthermore, the metallic corrosion products have the effect of catalyzing further oxidative breakdown of the oil.

A number of compounds, more especially those of the phenolic type, are known which exert an oxidation inhibiting effect when added to mineral lubricating oils and other hydrocarbon products. Their effect is to prevent oxidative breakdown of the oil both on storage (long potential reaction time and low temperature) and in use (short reaction time and high temperature). Although 35 many antioxidants are known which stabilize the oil adequately on storage, the majority of them tend to break down with undesirable rapidity at high engine operating temperatures.

A principal object of the present invention is to provide 45 a new class of lubricating oil antioxidants of good properties. Another object is to provide an antioxidant which is stable and effective at relatively high engine temperatures. Other objects and advantages will be apparent from the following description.

It has now been found, according to the present invention, that the salts formed by reacting thialdine or its homologs with xanthic and thioxanthic acids are extremely effective antioxidants for hydrocarbon products liable to oxidation, especially mineral lubricating oils.

Thialdine, otherwise known as 5,6-dihydro-2,4,6-trimethyl-1,3,5-dithiazine, is represented by the structural formula



It is readily prepared by treating the condensation product of acetaldehyde and ammonia with hydrogen sulfide. Thialdine and the homologs of the same which are useful

2

for the purposes of the present invention may be represented by the general formula



where R represents an alkyl group of 1 to 10 carbon atoms. However, simple thialdine in which R is methyl is preferred.

Acids which may be used in forming the thialdine salts of the present invention include xanthic acids of the formula ROCSSH and thioxanthic acids of the formula RSCSSH and are represented by the general formula



wherein X is selected from the group consisting of oxygen and sulfur and R represents an aliphatic radical having from 1 to 30 carbon atoms. The radical R' may be saturated or unsaturated, straight or branched chain, with or without cycloaliphatic substituent chains, or it may be an alkyl substituted cycloaliphatic nucleus. Examples of suitable alkyl and alkenyl xanthic and thioxanthic acids are the lower acids such as isopropyl, n-butyl, n-octyl, n-octylenyl, and n-decylenyl. Higher acids include dodecyl, hexadecyl, octadecyl, hexadecylenyl and the like. Mixtures of acids may be used. Aliphatic radicals having 2-20 carbon atoms are preferred. The most preferred products, however, are those prepared from the alkyl acids, both from the point of view of effectiveness and from the point of view of ease of preparation. The xanthic acids may be prepared by conventional means such as by reacting carbon disulfide with an alcohol or mercaptan having the desired hydrocarbon radical; usually the reaction is conducted in a KOH or NaOH solution of the alcohol or thioalcohol to prepare the stable potassium or sodium salt followed by hydrolysis to the xanthic acid by treatment with a mineral acid such as sulfuric acid. The acid may then be reacted with one mol of thialdine to give an addition product or salt.



65 The thialdine and homologous salts of the present invention may be readily formed by contacting the thialdine compound with the acid at a relatively low temperature such as 0 to 20°C. Since heat is evolved, the reaction is preferably conducted in the presence of an inert solvent and by contacting the reactants gradually, usually at temperatures as low as 0° to 5° C. Suitable solvents include chloroform, carbon tetrachloride,

ethylene dichloride, benzene, petroleum ether, and the like.

The following examples illustrate the preparation and testing of various thialdine salts according to this invention, but it is to be understood that these examples do not limit the scope of the invention in any way.

*Example I.—Preparation of thialdine isopropyl xanthate*

A solution of 34.8 grams (0.2 mol) of potassium isopropyl xanthate in 300 ml. of water was cooled to 5° C. after which 11.0 ml. of 50% H<sub>2</sub>SO<sub>4</sub> (0.1 mol) was added dropwise with rapid stirring in a 1-liter, 3-necked flask equipped with a stirrer, thermometer, and reflux condenser. The reaction temperature was maintained at 0° to 5° C.

A solution of 32.6 grams (0.20 mol) of thialdine in 500 ml. of petroleum ether was then added dropwise over a period of one hour to the isopropyl xanthic acid-containing solution, maintaining the temperature below 5° C. The organic layer was separated, dried over anhydrous Na<sub>2</sub>SO<sub>4</sub>, and placed on a steam bath to remove the solvent. A waxy, brown solid was obtained, which upon analysis was found to contain 40.0% sulfur, and 8.0% nitrogen.

*Example II.—Preparation of thialdine lauryl thioxanthate*

Lauryl thioxanthic acid was prepared by the method described in Example I, using 50.6 grams (0.16 mol) of potassium lauryl thioxanthate and 8.8 ml. of 50% H<sub>2</sub>SO<sub>4</sub> (0.08 mol).

The thialdine salt was also prepared by the method described in Example I, using 26.8 grams (0.16 mol) of thialdine. A viscous yellow oil was obtained which upon analysis was found to contain 33.0% sulfur, and 2.6% nitrogen.

*Example III.—Laboratory bearing corrosion tests*

In this test the additives were blended in 0.25% by weight concentrations in an extracted Mid-Continent oil of SAE 20 grade and comparative tests run on these blends and on a sample of the unblended oil. The test was conducted as follows:

500 cc. of the oil was placed in a glass oxidation tube 13 inches long and 2½ inches in diameter, fitted at the bottom with a ¼ inch air inlet tube perforated to facilitate air distribution. The oxidation tube was then immersed in a heating bath so that the oil temperature was maintained at 325° F. throughout the test. Two quarter-sections of automotive bearings of copper-lead alloy, of known weight and having a total surface area of 25 sq. cms., were attached to opposite sides of a stainless steel rod which was then immersed in the test oil and rotated at 600 R. P. M., thus providing sufficient agitation of the oil during the test. Air was then blown through the oil at the rate of 2 cu. ft. per hour. At the end of each four-hour period, the bearings were removed, washed with naphtha, and weighed to determine the amount of loss by corrosion. The bearings were then repolished (to increase the severity of the test), reweighed and then subjected to the test for additional four-hour periods in like manner. The results are given in the following table as "corrosion life," which indicates the number of hours required for the bearings to lose 100 mgs. in weight, determined by interpolation of the data obtained in the various periods.

| Thialdine Salt                             | Corrosion Life (hrs.) |
|--------------------------------------------|-----------------------|
| None (Base oil only)                       | 8                     |
| Thialdine Isopropyl Xanthate (Example I)   | 25                    |
| Thialdine Lauryl Thioxanthate (Example II) | 33                    |

*Example IV.—Lauzon engine test*

To confirm the results of this laboratory test under actual operating conditions, a further test was run using

an SAE 30 extracted Coastal oil containing 0.25 weight percent of the thialdine isopropyl xanthate of Example I as crankcase lubricant in a Lauzon engine. The operating conditions were 295° F. jacket temperature, 300° F. oil temperature, and 1800 R. P. M. at 1.5 indicated kilowatt load, and the duration of the test was 20 hours. At the end of the test the loss in weight of the copper-lead bearings was determined. A blank test was run for comparison, using the base oil alone. The results of the test are shown below.

| Oil                 | Weight Loss Per Bearing (mg.) |
|---------------------|-------------------------------|
| Base oil alone..... | 250                           |
| Blend.....          | 20                            |

From the preceding examples it will be evident that the thialdine salts of the present invention are effective antioxidants for lubricating oils.

As previously stated, any of the alkyl homologs of thialdine may be employed although thialdine itself is preferred.

The additives may be blended in the oil in amounts of from about 0.02 to 5% by weight, 0.5 to 2% being the preferred range. For load-bearing purposes quantities of 2 to 15% may be used. For handling and storage, concentrates containing 15 to 50% or more may be prepared. These may be added to base stocks to give blends of the desired concentration.

In addition to the additives of this invention there may also be added to the oil other conventional additives including detergent type additives, such as metal soaps, metal petroleum sulfonates, metal phenates, metal alcohates, metal alkyl phenol sulfides, and the like. Examples of such additional additives are barium tert-octyl phenol sulfide, calcium tert-amyl phenol sulfide, cadmium or nickel oleates, calcium phenyl stearate, aluminum naphthenate, and zinc methylcyclohexyl thiophosphate.

The lubricating oil base stocks used may be straight mineral lubricating oils or distillates derived from any suitable or desired crudes, or, if desired, blended oils may be employed. The oils may have been subjected to any conventional refining treatment such as acid, alkali and/or clay treatment, or solvent extraction. Synthetic oils such as those prepared by the polymerization of olefins or by the Fischer-Tropsch synthesis or those of the well known ether and ester type may alternatively be employed, alone, mixed, or in combination with mineral oils.

Further types of additives which may be present if desired include dyes, pour point depressants, heat thickened fatty oils, sulfurized fatty oils, organo-metallic compounds, sludge dispersers, thickeners, viscosity index improvers, oiliness agents, volatilized fats, waxes or oils, and colloidal solids such as graphite or zinc oxide, etc. Solvents, and assisting agents such as esters, ketones, alcohols, aldehydes, and halogenated or nitrated hydrocarbons may also be employed where necessary or desirable.

Particularly suitable assisting agents are the C<sub>8</sub> and higher alcohols (preferably C<sub>8</sub> to C<sub>12</sub>) such as lauryl and stearyl alcohols, and the "Oxo" alcohols of corresponding chain length.

In addition to being employed in lubricants, the additives of the present invention may also be employed in other hydrocarbon products susceptible to oxidative breakdown. Among these may be mentioned motor fuels, burning oils, mineral oil base hydraulic fluids, torque converter fluids, cutting oils, flushing oils, turbine oils, transformer oils, industrial oils and process oils, natural and synthetic hydrocarbon rubbers, and the like. They may also be used in gear lubricants, greases, and

in other products containing hydrocarbon oils as ingredients.

What is claimed is:

1. As a new composition of matter the salt formed by reacting a compound of the general formula

5



10

where R is a C<sub>1</sub> to C<sub>10</sub> alkyl radical, with an acidic compound of the general formula R'XCSSH where R' is selected from the group consisting of C<sub>1</sub> to C<sub>30</sub> aliphatic hydrocarbon radicals and X is selected from the group consisting of oxygen and sulfur.

2. A new composition of matter as in claim 1 wherein R' represents a monovalent aliphatic hydrocarbon radical of 2 to 20 carbon atoms.

3. Thialdine isopropyl xanthate.
4. Thialdine lauryl thioxanthate.

15

5. The process which comprises reacting a compound of the general formula



10

where R is a C<sub>1</sub> to C<sub>10</sub> alkyl radical, with an acidic substance selected from the group consisting of xanthic and thioxanthic acids at a temperature in the range of 0° to 20° C. and in the presence of an inert solvent.

15

References Cited in the file of this patent

UNITED STATES PATENTS

|           |              |       |               |
|-----------|--------------|-------|---------------|
| 2,084,011 | Teppema      | ----- | June 15, 1937 |
| 2,109,158 | Teppema      | ----- | Feb. 22, 1938 |
| 2,273,664 | Searle       | ----- | Feb. 17, 1942 |
| 2,439,734 | Himel et al. | ----- | Apr. 13, 1948 |
| 2,610,182 | McDermott    | ----- | Sept. 9, 1952 |

OTHER REFERENCES

Hackh's Chem. Dictionary, 3rd ed., page 848.